

Feb. 22, 1966

C. DOSTES ET AL

3,237,008

ROOMLIGHT HANDLING RADIOGRAPHIC ELEMENT INCLUDING  
AN X-RAY SENSITIVE LAYER OVERCOATED WITH A DYE  
DESENSITIZED SILVER HALIDE EMULSION  
Filed Jan. 19, 1961

**Fig. 1**



**Fig. 2**



**Claude Dostes  
Maurice E. Pfaff**

INVENTORS

BY *R. Frank Smith*  
*Lawrence H. Willis*

ATTORNEYS

1

3,237,008

## ROOMLIGHT HANDLING RADIOGRAPHIC ELEMENT INCLUDING AN X-RAY SENSITIVE LAYER OVERCOATED WITH A DYE DESENSITIZED SILVER HALIDE EMULSION

Claude Dostes, Joinville-le-Pont, Seine, and Maurice E. Pfaff, Eaubonne, Seine-et-Oise, France, assignors to Eastman Kodak Company, Rochester, N.Y., a corporation of New Jersey

Filed Jan. 19, 1961, Ser. No. 83,709

5 Claims. (Cl. 250—65)

This invention relates to photographic elements which have the light-sensitive layer or layers thereof protected from exposure to visible light. More particularly it relates to elements which are useful in obtaining X-ray photographs or radiograms. Still more particularly it relates to X-ray films which can be safely handled and processed under conditions of ordinary room-light illumination without exposure of the photosensitive layers thereof.

There have been various methods proposed in the art for protecting the light-sensitive layer or layers of photographic elements used in obtaining X-ray photographs. Certain of these photographic elements have been provided with an opaque protecting medium which is removed after exposure in a special processing bath. Such protective layers have not been entirely satisfactory because the layers are difficult to remove after exposure to X-rays and the light-blocking material is not always uniformly distributed throughout the medium. Other photographic elements have been prepared using protective outer-layers, comprising a coating of chrome-yellow, Venetian red, and the like which forms a readily removable opaque protecting medium. This coating allows handling of the element in ordinary room light but is washed off prior to development so that development must of necessity be carried out in a darkroom. With any of the prior proposals for protecting the light-sensitive layer using an outer-protective opaque layer, there has also been the difficulty that these protective layers do not cover the edges of the film, and accordingly, light enters the film through these edges to produce edge-fog in the light-sensitive emulsion layer. To overcome this difficulty, it has been proposed to optically seal the edges of the film by applying a black colloid edge-coating or a sealing strip of opaque paper or fabric. It is apparent that the prior art has been unable to deduce a method for preparing a truly satisfactory roomlight handling photographic element. To meet the requirements of such an element, it should be stable to visible light exposure but have substantially unchanged sensitivity to X-ray radiation. The element should also be stable against edge-fog without requiring special treatment or expensive extra handling of separate film sheets to employ special optical sealers, light-blocking cassettes, etc. The roomlight handling elements should also be adapted to processing in conventional processing solutions without loss of optimum quality in the final result. It will be apparent from a reading of the present specification and claims that we have found, quite unexpectedly, a way to prepare roomlight handling photographic elements which meet each of the above requirements while at the same time allowing the operator to watch the complete development process under ordinary room light.

It is therefore an object of the present invention to provide a photographic element for X-rays which can be handled under conditions of ordinary roomlight illumination. A further object is to provide roomlight handling radiographic elements which are stable against edge fog. A still further object is to provide an element which can be processed in room light using conventional processing

2

solutions. Another object is to provide roomlight handling radiographic elements which have light-blocking outer protective layers which permit observation of image development in ordinary room light. Another and still further object is to provide such elements wherein the light-absorbing materials are readily removed in conventional fixing baths. Other objects will appear hereinafter.

According to the present invention the roomlight handling radiographic element carries an outer emulsion layer which is a light-blocking layer for the inner-most light sensitive, X-ray sensitive emulsion layer. The objects of the invention are accomplished by incorporating in each of the emulsion layers of the roomlight handling photographic element, a combination of a nitrogen-containing heterocyclic silver halide desensitizing compound and a yellow dye which absorbs a substantial portion of the visible radiation to which the silver halide is sensitive (i.e., radiation between about 350 and 500 mu). According to the present invention, the desensitizing compounds should be capable of strongly depressing the light sensitivity of the silver halide without appreciably affecting the X-ray sensitivity. The desensitized silver halide grains should be readily removed from the layers of the radiographic elements in conventional processing baths. The dyes used in each layer should also be readily removed or decolorized in conventional processing solutions. In the outermost light-blocking layer, the strongly desensitized silver halide should be readily removed in conventional processing solutions but not until development of the innermost layer has occurred. After roomlight processing, both the silver halide and the incorporated dye should be removed from all layers or decolorized leaving a clearly visible radiographic image.

By reference to the accompanying drawing, there can be seen the manner in which the roomlight handling radiographic elements of our invention can be prepared. FIG. 1 shows a sectional view of a photographic element having a light-sealing backing layer, whereas FIG. 2 shows an element which has an X-ray sensitive layer and a light-blocking layer on each side of the single support.

The nitrogen-containing heterocyclic silver halide desensitizing compounds which are useful in the practice of our invention can advantageously be represented by the following structural formulas:





6-ethoxy-2-(m-nitrostyryl) quinolinium ethylethosulfate



3,7-diamino-5-phenyl-phenazinium chloride



5-nitrobenzimidazole

Additional useful nitrogen-containing heterocycles representative of the above classes comprise the following:



2-(o-nitrostyryl)-3-ethylbenzothiazolium iodide,  
2-(o,p-dinitrostyryl)-benzothiazole,  
6-nitro-benzo-1,2,3-triazole,  
4-chloro-benzo-1,2,3-triazole,



5-chloro-benzo-1,2,3-triazole,  
2-methyl-6-nitrobenzothiazole metho-p-toluenesulfonate,  
2-(p-nitrostyryl)-quinoline metho-p-toluenesulfonate,  
4-(p-nitrostyryl)-quinoline methiodide,  
1-ethyl-7-nitro-quinolinium ethylsulfate,  
1,3-diamino-5-methylphenazinium chloride,  
1,3-diamino-5-benzylphenazinium chloride,  
3,7-diamino-5β-hydroxy-ethylphenazinium chloride,  
5-chlorobenzimidazole,  
2-methyl-5-chlorobenzimidazole,  
2-mercaptopbenzimidazole,  
2-mercapto-6-chlorobenzimidazole.

The desensitizing compounds of the above type which can be advantageously employed in practicing our invention have been described in one or more of the following representative U.S. Patents: 2,400,872, May 28, 1946; 2,541,472, February 13, 1951; 2,939,789, June 7, 1960; 2,915,395, December 1, 1959; and 2,066,099, December 29, 1936.

The visible-light absorbing dyes which are used in combination with the desensitizing compounds of this invention in the silver halide emulsion layers should advantageously be dyes which are stable in a colloid carrier and should advantageously be nondiffusing. To be suitable, they should be readily removable in the customary processing baths, or be decolorized entirely by the con-

ventional processing solutions. Suitable dyes should also be highly absorbent in the regions of the spectrum to which the emulsion is sensitive, but should transmit the rest of the visible spectrum freely so that it is possible to observe the progress of development under ordinary room light.

According to the present invention, we have found that the yellow-colored dyes containing a styryl nucleus, and 5-pyrazolone dyes are suitable for the purpose and meet each of the above requirements.

Suitable styryl nucleus-containing dyes comprise the following:

(1) 2(2'-methoxystyryl) quinoline hydrochloride



(2) 2(4'-methoxystyryl) quinoline hydrochloride



(3) The condensation product from two molecular proportions of quinaldine methylsulfate and one molecular proportion of 4:4'-diphenyl dialdehyde in pyridine: The yellow-colored product of the probable formula:



(4) The condensation product from two molecular proportions of quinaldine dimethylsulfate and one molecular proportion of azoxy benzalaniline in pyridine: The yellow-colored product of the probable formula:



(5) The styryl-containing condensation product from quinaldine-methylsulfate and piperonal:



(6) The styryl-containing condensation product from quinaldine-methylsulfate and veratric aldehyde:



(7) The styryl-containing condensation product from quinaldine-methylsulfate and anisaldehyde:



(8) The styryl-containing condensation product from 2-methyl-3-methylbenzothiazole-methylsulfate with p-ami-

no-benzaldehyde and reacted with undecoylchloride in the presence of pyridine and having the probable formula:



(9) The styryl-containing condensation product from 2-methyl-thiazoline-dimethyl-sulfate and p-amino-benzaldehyde, reacted with undecylenic acid chloride in the presence of methylamine and having the probable formula:



(10) 4 (phenylazo)-5-pyrazolone-3-carboxylic acid calcium salt having the formula:



prepared according to the disclosure of U.S. Patent 2,503,717, issued April 11, 1950.

(11) 4,4' - methenyl-bis-(1-naphthyl-3-methyl-pyrazolone-5) of the formula:



(12) 3 - carboxy-1-(1'-sulfophenyl)-4-(4''-sulfophenylazo)-5-pyrazolone, disodium salt:



Other 5-pyrazolone dyes of the type suitable for use in the present invention comprise bis[1-(p-sulfophenyl)-3-methyl - 5-pyrazolone-(4)]-methinoxonol; bis[1-(p-sulfophenyl) - 3 - methyl-5-pyrazolone-(4)]trimethinoxonol; bis - [3 - methyl-1-p-sulfophenyl-5-pyrazolone-(4)]pentamethinoxonol; and others as disclosed in U.S. Patent 2,852,386, issued September 16, 1958.

The yellow-colored dyes of Formulas 1 and 2 can be prepared by heating styryl quinoline containing a reactive methyl group with a substituted aromatic aldehyde in the presence of anhydrous zinc chloride in a sealed tube at 100° C. for several hours. After the heat treatment, the product is treated with hydrochloric acid and hot water, filtered and made alkaline with ammonia. The precipitated styryl derivative of the base can then be recrystallized and converted to the salt by the addition of acid.

The light-absorbing compounds of the above type which can be advantageously employed in practicing our invention have been described herein or are described in one or more of the following representative patents: U.S. 2,274,782, March 3, 1942; 2,503,717, April 11, 1950; 2,058,725,

October 27, 1936; 2,186,731, January 9, 1940; 1,845,404, February 16, 1932; and British 399,387, October 5, 1933.

According to our invention, we incorporate in each silver halide emulsion layer of the roomlight handling element one or more of the desensitizing compounds with one or more visible light-absorbing compounds, each of which are represented hereinabove. The desensitizing compounds and the visible light-absorbing materials can be contained in combination in various concentrations in the layers of the roomlight handling radiographic elements.

Ordinarily in the innermost layer which is X-ray sensitive and also light sensitive, we employ a desensitizing compound in the order of from about 3.0 mg. to about 300 mg. per mole of silver halide. The light-absorbing dye of the styryl-nucleus-containing type is added to the emulsion in a concentration in the order of from about 0.5 to about 5.0 grams per mole of silver halide and dyes of the 5-pyrazolone type are added to the emulsion in the range from about 10 to about 100 grams per mole of silver halide.

The outer-light-blocking protective layer normally comprises a silver halide emulsion layer more strongly desensitized than is the innermost light-sensitive layer. In the outermost layer, we normally employ an excess of desensitizing compound, this can be in the order of from about 20 mg. to 5.0 grams per mole of silver halide or more depending to some extent upon the desensitizing compound employed. The visible light-absorbing dye is added in combination with the desensitizing compound in the emulsion in an amount from about 0.5 to about 5.0 grams per mole of silver halide for styryl-nucleus-containing dyes and from about 10 to 100 grams per mole of silver halide for the 5-pyrazolone dyes. In the outer-light-blocking emulsion layer a suitable concentration of silver per square foot can vary from about 100 to about 900 mg. of silver per square foot.

The outer-light protecting emulsion layer can comprise a silver halide emulsion which forms latent images predominantly inside the silver halide crystal, such as those described in Davey and Knott, U.S. Patent 2,592,250, issued April 8, 1952. Where emulsions of this type are used according to the invention, desensitizing compounds of the type herein described are incorporated in an amount in the range from about 25 mg. to about 250 mg. per mole of silver halide. In such emulsion layers the light-absorbing dyes are contained in combination with desensitizing compounds in the range as indicated above for outer-light-blocking layers.

50 Silver halide emulsions which form latent images predominantly inside the silver halide crystal are also referred to as internal image emulsions and have been described in the co-pending application of Luckey et al., U.S. patent application Serial No. 786,225, filed January 12, 1959, now U.S. Patent 2,996,382, issued on August 15, 1961. The internal image emulsions which are useful according to our invention have a reduced surface sensitivity. Such internal image emulsions, when measured according to normal photographic techniques by coating a test portion of the emulsion on a transparent support, exposing to a light-intensity scale having a fixed time between 0.01 and 1 second, bleaching 5 minutes in a 0.3 percent potassium ferricyanide solution at 65° F., and developing for about 5 minutes at 65° F. in developer B below, has a sensitivity, measured at a density of 0.1 above fog, appreciably greater (e.g., at least 1.4 log E greater) than the sensitivity of an identical test portion which has been exposed in the same way and developed for 6 minutes at 68° F. in developer A below.

70 The developer compositions which are used in defining an internal image emulsion by comparison with a conventional surface image emulsion developer, compositions A and B are given hereinafter. Developer A is the usual type of surface image developer and developer B is an internal developer having high silver halide solvent activity.

The following developer compositions are used in the method of determining relative internal sensitivity of preferred emulsions:

| (A):                           | Grams | 5  |
|--------------------------------|-------|----|
| N-methyl-p-aminophenol sulfate | 0.31  |    |
| Sodium sulfite, desiccated     | 39.6  |    |
| Hydroquinone                   | 6.0   |    |
| Sodium carbonate, desiccated   | 18.7  |    |
| Potassium bromide              | 0.86  | 10 |
| Citric acid                    | 0.68  |    |
| Potassium metabisulfite        | 1.5   |    |
| Water to make 1.0 liter.       |       |    |
| (B):                           |       |    |
| N-methyl-p-aminophenol sulfate | 2.0   | 15 |
| Sodium sulfite, desiccated     | 90.0  |    |
| Hydroquinone                   | 8.0   |    |
| Sodium carbonate, monohydrate  | 52.5  |    |
| Potassium bromide              | 5.0   |    |
| Sodium thiosulfate             | 10.0  | 20 |
| Water to make 1.0 liter.       |       |    |

Suitable internal image emulsions are described in Davey and Knott, U.S. Patent 2,592,250, issued April 8, 1952. Other emulsions which can be used in the outermost layers of the present invention comprise, for example, relatively insensitive silver chlorobromide and silver bromoiodide emulsions.

The methods of incorporating the desensitizing compounds and visible light-absorbing materials in silver halide emulsions are well known to those skilled in the art. The desensitizing compounds can be directly dispersed in the emulsions, or they can be dissolved in water (or in organic solvents, such as methanol, ethanol, etc., where the water-solubility is not sufficiently great) and added in the form of their solutions. While the visible light-absorbing dyes can be directly dispersed in the emulsions, it is convenient to add the same in the form of solutions in appropriate solvents. Methanol, ethanol, pyridine, and the like have proved satisfactory for many of the dyes herein disclosed. Mixtures of solvents, e.g., pyridine diluted with methanol or acetone, can also be used. According to the invention the desensitizing compounds and the visible light-absorbing dyes are dispersed in the finished emulsions and should be uniformly distributed throughout the emulsions. The following procedure is satisfactory:

Stock solutions of the desensitizing compounds and visible light-absorbing dyes are prepared by dissolving the same in appropriate solvents as described above. The desired amount of the stock solution of one of the dyes (or desensitizing compounds) is slowly added to the liquid gelatino-silver halide emulsion with stirring. Stirring is continued until the dye is thoroughly incorporated in the emulsion. Then the desired amount of the stock solution of the desensitizing compound (or dye, if the desensitizing compound has been added first) is slowly added to the emulsion, while stirring. Stirring is continued until the second solution is thoroughly incorporated. The treated emulsion can then be coated out on a suitable support, such as glass, cellulose derivative film, resin film, or paper, to suitable thicknesses and allowed to dry. Most usually the roomlight handling radiographic elements of our invention are dupli coated, i.e., coated on either side of a support with the light-sensitive, X-ray-sensitive emulsion layer being the innermost layer, and the light protecting outer layer being coated as a second layer on either side of the support. The details of such coating methods are well known to those skilled in the art and have been described in U.S. Patent 1,947,160, issued February 13, 1934.

The coating thickness of the innermost light-sensitive, X-ray-sensitive layer of the multilayer radiographic elements prepared according to the invention can vary widely, but in general thicknesses from about 0.4 to about 1.2 mils, can be used. The thicknesses of the outer-protective layers are not critical and can depend more upon the con-

centration of the light diffusing, e.g., silver halide, and absorbing materials per square foot of coated surface.

The following examples will serve to illustrate further the present invention.

#### EXAMPLE 1

To a liquid coarse grain gelatino-silver bromoiodide emulsion, prepared in the usual manner, was added per mole of silver halide, 50 mg. of 2-methyl-5-nitrobenzothiazole metho-p-toluenesulfonate (I) and 0.5 gram of 2-(2'-methoxystyryl)quinoline hydrochloride (II). Thereafter the emulsion was coated at 90° F. according to U.S. Patent 1,947,160, issued February 13, 1934, on both sides of an ordinary cellulose acetate film, and dried.

On either side of the coated support in the same manner an internal image emulsion was coated which was prepared according to the disclosure of U.S. Patent 2,592,250, issued April 8, 1952, into which had been added with stirring 50 mg. of compound I and 0.5 gram of compound II per mole of silver halide. The additions to the emulsion were made while holding at 90° F. The emulsion composition was coated at 90° F. at a thickness to give 600 mg. of silver halide per square foot, and dried.

The resulting film was exposed to an 80 kv. X-ray source under roomlight illumination, developed in a bath of the composition of Table 1, fixed, and washed. All of the steps for processing of the roomlight handling radiographic element of this example were carried out under ordinary roomlight illumination. The radiogram produced by this example was of good quality and did not show evidence of edge fog.

In the present invention the speed of the innermost layer can advantageously be from about 50 to about 100 times that of the outer-light blocking layer when developed in a surface developer, such as developer A above.

Table 1

|                               |       |      |
|-------------------------------|-------|------|
| Water at 125° F.              | cc    | 500  |
| N-methyl-p-aminophenolsulfate | grams | 2.0  |
| Sodium sulfite (desiccated)   | do    | 90.0 |
| Hydroquinone                  | do    | 8.0  |
| Sodium carbonate monohydrate  | do    | 52.5 |
| Potassium bromide             | do    | 5.0  |
| Water to make 1.0 liter.      |       |      |

#### EXAMPLE 2

A clean cellulose acetate film base was coated according to Example 1 with a coarse grain silver bromoiodide emulsion prepared in the usual manner which had been desensitized with 43.5 mg. of 4-nitro-6-chlorobenzotriazole (I) and to which was added 25 grams of 3-carboxy-1-(1'-sulfophenyl)-4-(4"-sulfophenylazo)-5-pyrazolone disodium salt (II) per mole of silver halide. The silver content of the coating was 882 mg. per square foot. As an outer-light-blocking layer a fine-grain, silver bromoiodide emulsion strongly desensitized with 900 mg. of compound I and containing 80 grams of compound II per mole of silver halide was coated over each of the light-sensitive, X-ray-sensitive layers at a thickness to give 540 mg. of silver per square foot.

After drying the coated film was handled for 15 minutes under 40-foot candles of cool light fluorescent illumination during exposure of the film to an 80 kv. X-ray source and developed in a developer composition of Example 1 to produce a radiogram of good contrast and speed and without the formation of edge fog.

#### EXAMPLE 3

An ordinary cellulose acetate film base was coated on either side as shown in Example 2 with a coarse grain silver bromoiodide emulsion prepared in the usual manner which was desensitized with 50 mg. of 6-ethoxy-2-(m-nitrostyryl)quinolinium ethylethosulfate (I) and to which was added 2.5 grams of 2-(4'-methoxystyryl)quinoline hydrochloride (II) per mole of silver halide. The silver content of the coating was 750 mg. per square foot.

As an outer-light-blocking layer a silver bromide emulsion containing some silver iodide prepared according to U.S. Patent 2,592,250 was desensitized with 50 mg. of compound I and to which was added 1 gram of compound II per mole of silver halide. The outer-light-blocking layer was coated over each of the light-sensitive layers according to Example 2 at a thickness to give 500 mg. of silver per square foot.

The roomlight handling radiographic element was thereafter exposed and processed in room light for five minutes in a developer of Table 2. The progress of development was watched under roomlight illumination during processing.

Table 2

|                                | Grams |
|--------------------------------|-------|
| N-methyl-p-aminophenolsulfate  | 2.2   |
| Hydroquinone                   | 8.8   |
| Sodium sulfite (anhydrous)     | 72.0  |
| Sodium carbonate (crystalline) | 130.0 |
| Potassium bromide              | 4.0   |
| Water to make 1.0 liter.       |       |

The exposed and developed film was then fixed in a well-known manner, washed, and dried. The resulting radiogram was of good quality and showed substantially no edge fog.

Alternatively, the innermost and outermost coatings of the roomlight-handling radiographic elements can contain other visible light-absorbing dyes. For example: merocyanine dyes such as those described by Brooker et al., U.S. Patent 2,493,747, issued January 10, 1950. The outer light-absorbing pigments in the outer-light-blocking layers of our invention can also comprise light-absorbing pigments such as zinc oxide, lead chromate, silver chromate, the silver salt of dyes derived from thiobarbituric acid as described by A. H. Herz in U.S. Patent 2,719,088, issued September 27, 1955, and tartrazine mordanted with polyvinyl pyrrolidone. In accordance with our invention, it is possible to use a light filtering layer between the innermost layer and the outermost protective layer to prevent diffusion of additive materials which might otherwise become introduced into the innermost X-ray sensitive layer. For example, a suitable interlayer to prevent diffusion of acid dyes was found to comprise polyvinyl- $\alpha$ -methyl-allyl-N-quanidyl ketime and other suitable compounds in gelatin as described in U.S. Patent 2,882,156, issued April 14, 1959.

Our invention will now be described by reference to the accompanying drawing. In FIG. 1 the support 10 is coated with a light-sensitive, X-ray-sensitive layer 11 which has coated thereon a light-blocking silver halide emulsion layer 12 which prevents the exposure of the light-sensitive layer 11 during roomlight handling of the radiographic element. On the back side of the element there is coated a light-sealing backing layer 13. The backing layers suitably employed in the invention must be antihalation layers which dissolve smoothly in photographic developers and which do not disintegrate and contaminate conventional developer solutions, such as described in U.S. Patent 2,327,828, issued August 24, 1943.

In FIG. 2 of the accompanying drawing the support 10 is coated on each side with an X-ray-sensitive, light-sensitive layer 11 and superimposed on each of the light-sensitive layers are the light-blocking silver halide emulsion layers 12. In roomlight handling element of the type shown in FIG. 2, a light-sealing backing layer is not used since the outer protective layers protect the innermost layers 11 from visible light exposure.

The invention has been described in detail with particular reference to preferred embodiments thereof, but it will be understood that variations and modifications can be effected within the spirit and scope of the invention as described hereinabove and as defined in the appended claims.

We claim:

1. A roomlight handling photographic element comprising a support having coated thereon at least one X-ray-sensitive gelatino-silver halide emulsion layer containing about 3 milligrams to 300 milligrams of a nitrogen-containing heterocyclic silver halide desensitizing compound per mole of silver halide and a yellow dye selected from the group consisting of styryl-nucleus containing dyes at a concentration of about .5 gram to 5 grams per mole of silver halide and 5-pyrazolone dyes at a concentration of about 10 grams to 100 grams per mole of silver halide, and coated on said X-ray-sensitive layer at least one light-blocking gelatino-silver halide emulsion layer more strongly desensitized than said X-ray-sensitive layer and containing about 20 milligrams to 5 grams of a nitrogen-containing heterocyclic silver halide desensitizing compound per mole of silver halide and a yellow dye selected from the group consisting of styryl-nucleus containing dyes at a concentration of about .5 gram to 5 grams per mole of silver halide and 5-pyrazolone dyes at a concentration of about 10 grams to 100 grams per mole of silver halide, said yellow dye being absorbent in the regions of the visible spectrum in which said gelatino-silver halide emulsions are sensitive and suitable to transmit the rest of the visible spectrum so that the progress of development of said X-ray-sensitive layer can be observed in roomlight.

2. A roomlight handling photographic element comprising a support having coated on both sides thereof an X-ray-sensitive gelatino-silver halide emulsion layer containing about 3 milligrams to 300 milligrams per mole of silver halide of a nitrogen-containing heterocyclic silver halide desensitizing compound and a yellow dye selected from the group consisting of styryl-nucleus containing dyes at a concentration of about .5 grams to 5 grams per mole of silver halide and 5-pyrazolone dyes at a concentration of about 10 grams to 100 grams per mole of silver halide, and superimposed on each of said X-ray-sensitive layers a light-blocking gelatino-silver halide emulsion layer wherein the silver halide forms latent images predominantly inside the silver halide crystals more strongly desensitized than said X-ray-sensitive layers and containing about 25 milligrams to 250 milligrams per mole of silver halide of a nitrogen-containing heterocyclic silver halide desensitizing compound and a yellow dye selected from the group consisting of styryl-nucleus containing dyes at a concentration of about .5 gram to 5.0 grams per mole of silver halide and 5-pyrazolone dyes at a concentration of about 10 grams to 100 grams per mole of silver halide, said yellow dye being absorbent in the regions of the visible spectrum in which said gelatino-silver halide emulsions are sensitive and suitable to transmit the rest of the visible spectrum so that the progress of development of said X-ray-sensitive layers can be observed in roomlight.

3. A roomlight handling photographic element comprising a support having coated on both sides thereof an X-ray-sensitive gelatino-silver halide emulsion layer containing about 3 milligrams to 300 milligrams per mole of silver halide of 2-methyl-5-nitrobenzothiazole metho-p-toluenesulfonate and about .5 gram to 5 grams per mole of silver halide of 2(2'-methoxystyryl)quinoline hydrochloride, and superimposed on each of said X-ray-sensitive layers a light-blocking gelatino-silver halide emulsion layer that forms latent images predominantly inside the silver halide crystals more strongly desensitized than said X-ray-sensitive layers and containing about 20 milligrams to 5 grams per mole of silver halide of 2-methyl-5-nitrobenzothiazole metho-p-toluenesulfonate and about .5 gram to 5 grams per mole of silver halide of 2(2'-methoxystyryl)quinoline hydrochloride, said yellow dye being absorbent in the regions of the visible spectrum in which said gelatino-silver halide emulsions are sensitive and suitable to transmit the rest of the visible

spectrum so that the progress of development of said X-ray-sensitive layer can be observed in roomlight.

4. A roomlight handling photographic element comprising a support having coated on both sides thereof an X-ray-sensitive gelatino-silver halide emulsion layer containing about 3 milligrams to 300 milligrams per mole of silver halide of 4-nitro-6-chlorobenzotriazole and about 10 grams to 100 grams per mole of silver halide of 3-carboxy-1-(1'-sulfophenyl)-4-(4"-sulfophenylazo)-5-pyrazolone disodium salt, and having superimposed on each of said X-ray-sensitive layers a light-blocking gelatino-silver halide layer more strongly desensitized than said X-ray-sensitive layers containing about 20 milligrams to 5 grams per mole of silver halide of 4-nitro-6-chlorobenzotriazole and about 10 grams to 100 grams per mole of silver halide of 3-carboxy-1-(1'-sulfophenyl)-4-(4"-sulfophenylazo)-5-pyrazolone disodium salt, said yellow dye being absorbent in the regions of the visible spectrum in which said gelatino-silver halide emulsions are sensitive and suitable to transmit the rest of the visible spectrum so that the progress of development of said X-ray-sensitive layer can be observed in roomlight.

5. A roomlight handling photographic element comprising a support having coated on both sides thereof an X-ray-sensitive gelatino-silver halide emulsion layer containing about 3 milligrams to 300 milligrams per mole of silver halide of 6-ethoxy-2-(m-nitrostyryl)quinolinium ethylethosulfate and about .5 gram to 5 grams per mole of silver halide of 2(4'-methoxystyryl)quinoline hydrochloride, said yellow dye being absorbent in the regions of the visible spectrum in which said gelatino-silver halide emulsions are sensitive and suitable to transmit the rest of the visible spectrum so that the progress of development of said X-ray-sensitive layer can be observed in roomlight.

ray-sensitive layers containing about 20 milligrams to 5 grams per mole of silver halide of 6-ethoxy-2-(m-nitrostyryl)quinolinium ethylethosulfate and about .5 gram to 5 grams per mole of silver halide of 2(4'-methoxystyryl)quinoline hydrochloride, said yellow dye being absorbent in the regions of the visible spectrum in which said gelatino-silver halide emulsions are sensitive and suitable to transmit the rest of the visible spectrum so that the progress of development of said X-ray-sensitive layer can be observed in roomlight.

10

## References Cited by the Examiner

## UNITED STATES PATENTS

|           |         |                |        |
|-----------|---------|----------------|--------|
| 2,090,607 | 8/1937  | Baldsiefen     | 96—101 |
| 2,098,442 | 11/1937 | Troland        | 96—108 |
| 2,503,717 | 4/1950  | Fierke et al.  | 96—84  |
| 2,541,472 | 2/1951  | Kendall et al. | 96—101 |
| 2,542,304 | 2/1951  | Boucher        | 250—68 |
| 2,592,250 | 4/1952  | Davey et al.   | 96—94  |
| 2,725,296 | 11/1955 | Kendall        | 96—68  |
| 2,759,822 | 8/1956  | Jones et al.   | 96—68  |
| 2,853,386 | 9/1958  | Tong           | 96—114 |
| 2,882,156 | 4/1959  | Minsk          | 96—114 |
| 3,114,833 | 12/1963 | Fine           | 96—68  |

## FOREIGN PATENTS

|         |        |          |
|---------|--------|----------|
| 230,964 | 2/1911 | Germany. |
| 334,878 | 3/1921 | Germany. |

30 NORMAN G. TORCHIN, Primary Examiner.

RALPH G. NILSON, Examiner.